

Jan. 24, 1967

A. C. SMITH, JR

3,300,307

PHOTOGRAPHIC DEVELOPER COMPOSITION

Filed Jan. 18, 1963

**Fig. 1**



**Fig. 2**



**Fig. 3**



ALBERT C. SMITH, JR.  
INVENTOR.

*R. Frank Smith*  
BY  
*Henry E. Byers*  
ATTORNEYS

1

3,300,307

**PHOTOGRAPHIC DEVELOPER COMPOSITION**  
Albert C. Smith, Jr., Rochester, N.Y., assignor to Eastman Kodak Company, Rochester, N.Y., a corporation of New Jersey

Filed Jan. 18, 1963, Ser. No. 252,340  
6 Claims. (Cl. 96—36)

This invention relates to tanning photographic developers and particularly to silver halide emulsions containing tanning developers.

Many photographic silver halide developers are recognized as tanning developers including hydroquinone, catechol and the like. For instance, 4-phenyl catechol has been incorporated in emulsions as disclosed in Yackel, U.S. Patent 2,592,368 issued April 8, 1952. However, this developer must be dissolved in a coupler solvent and then used as a dispersion in the photographic emulsion. For some purposes, the presence of the coupler solvent tends to make the final coatings softer than desirable. Moreover, the preparation of the dispersion for addition to the emulsion requires colloid which increases the total amount of colloid in the coated emulsion. This is undesirable where the coatings should be thin and relatively hard. For these reasons, it has been desirable to find a tanning developing agent which could be incorporated into photographic emulsions which would not require the use of a coupler solvent but would provide satisfactory hardening action, so that wash-off relief images can be obtained following customary silver halide developing.

Replacing 4-phenyl catechol with one of the more common, water soluble developer agents such as hydroquinone, catechol, or gallic acid has not resulted in obtaining a suitable wash-off relief image. Moreover, the oxidation products of these developers are colored and would produce stain when incorporated in a relatively thin wash-off relief type photographic emulsion. Therefore, the requirements for a suitable incorporated developer have been stringent.

I have found a silver halide tanning developer combination which is water soluble and can be added directly to the silver halide emulsion, but which has colorless oxidation products and is relatively free from staining.

One object of this invention is to provide a new tanning developer. Another object is to provide a photographic emulsion which contains a tanning developer but which results in a relatively hard wash-off relief image and is free from staining. A further object is to provide a combination of gentisic acid with an auxiliary developing agent which can be used in a tanning developer containing silver halide photographic emulsion. Additional objects will be apparent from the following disclosure.

The above objects are obtained by adding to a light-sensitive silver halide emulsion a combination of gentisic acid and an auxiliary developing agent. A useful concentration range for the gentisic acid is from about 10 to 150 grams, with a preferred range of from about 25 to 75 grams per mole of silver. A useful concentration for the auxiliary developing agent is from about 1 to 25 grams, with a preferred range of from about 2.5 to 10 grams per mole of silver.

Various auxiliary developing agents are known in the art and may be used with gentisic acid, but the preferred auxiliary developing agent is a substituted 3-pyrazolidone having the following general structure



2

in which the R groups each represent various substituents such as hydrogen, alkyl or aryl groups, for example, R<sub>1</sub> can be hydrogen or a group such as alkyl preferably containing from 1 to 4 carbon atoms, or an aryl group of the benzene or naphthalene series substituted or not, and R<sub>2</sub>, R<sub>3</sub>, R<sub>4</sub> and R<sub>5</sub> can be hydrogen atoms, or groups such as an alkyl group preferably of 1 to 4 carbon atoms or aryl such as phenyl.

The following compounds are representative of 3-pyrazolidone silver halide auxiliary developing agents which are useful in the developer compositions of the invention:

- (1) 1-phenyl-3-pyrazolidone
- (2) 1-p-tolyl-3-pyrazolidone
- (3) 5-phenyl-3-pyrazolidone
- (4) 5-methyl-3-pyrazolidone
- (5) 1-p-chlorophenyl-3-pyrazolidone
- (6) 1-phenyl-5-phenyl-3-pyrazolidone
- (7) 1-m-tolyl-3-pyrazolidone
- (8) 1-phenyl-5-methyl-3-pyrazolidone
- (9) 1-p-tolyl-5-phenyl-3-pyrazolidone
- (10) 1-m-tolyl-3-pyrazolidone
- (11) 1-p-methoxyphenyl-3-pyrazolidone
- (12) 1-acetamidophenyl-3-pyrazolidone
- (13) 1-phenyl-2-acetyl-4,4-dimethyl-3-pyrazolidone
- (14) 1-phenyl-4,4-dimethyl-3-pyrazolidone
- (15) 1-m-aminophenyl-4-methyl-4-propyl-3-pyrazolidone
- (16) 1-o-chlorophenyl-4-methyl-4-ethyl-3-pyrazolidone
- (17) 1-m-acetamidophenyl-4,4-diethyl-3-pyrazolidone
- (18) 1-p-( $\beta$ -hydroxyethylphenyl)-4,4-dimethyl-3-pyrazolidone
- (19) 1-p-hydroxyphenyl-4,4-dimethyl-3-pyrazolidone
- (20) 1-p-methoxyphenyl-4,4-diethyl-3-pyrazolidone
- (21) 1-p-tolyl-4,4-dimethyl-3-pyrazolidone
- (22) 1-(7-hydroxy-2-naphthyl)-4-methyl-4-n-propyl-3-pyrazolidone
- (23) 1-p-diphenyl-4,4-dimethyl-3-pyrazolidone
- (24) 1-p-( $\beta$ -hydroxyethylphenyl)-3-pyrazolidone
- (25) 1-o-tolyl-3-pyrazolidone
- (26) 1-o-tolyl-4,4-dimethyl-3-pyrazolidone

The following examples are intended to illustrate our invention but not to limit it in any way.

*Example I*

An unhardened gelatin fine-grain silver chloride photographic emulsion which contained a coating aid and a pyrazolidone developing agent was split into two portions. Hydroquinone was added to Portion A and gentisic acid was added to Portion B. Both portions were coated on a paper base. Samples of these coatings were given a reflex exposure to a line copy and immersed in a 4% sodium carbonate activator for one minute and then washed in 90° F. water. It was found that the sample containing gentisic acid produced sharper and more uniform images than did the hydroquinone-containing sample. It was noticed the hydroquinone-containing coating was very susceptible to aerial oxidation when wet with the alkaline solution, and it exhibited decreased activity after storage.

When samples of the above coatings were held for several weeks and then exposed, activated, and washed it was observed that the gentisic-containing coating gave results similar to that of the fresh coating; whereas, the hydroquinone-containing coating, due to the solubility, vapor pressure, etc., of the hydroquinone, showed poor developability, undesirable stain, etc., which indicated that the hydroquinone did not remain in the emulsion layer during storage but tended to sublime out of the element and wander to other samples in close contact with the element containing the incorporated hydroquinone.

*Example II*

An unhardened gelatin silver chloride emulsion which contained a coating aid and a 3-pyrazolidone developing agent was divided into several portions. Gentisic acid was added to one portion while either gallic acid, pyrogallol or catechol were added to other portions of the emulsion. The emulsion samples were then coated on a suitable support and dried. Samples of each of these coatings were tested as described in Example I above. The gentisic acid coating produced processed samples of good uniformity which were free of stain; whereas, the samples containing either gallic acid, pyrogallol or catechol, due to their instability and solubility under these conditions, exhibited poor uniformity and/or disadvantageous stain.

*Example III*

An unhardened gelatin silver halide photographic emulsion (predominantly silver chloride), containing one mole of silver halide, 340 grams of gelatin and 5700 grams of water, was jelled, noodled, and washed for one-half hour with water then melted at 40° C. and the following additions made:

650 grams of 8% aqueous saponin solution  
 680 grams of dispersion A (A dispersion of 4-phenyl catechol prepared by dissolving 50 grams of 4-phenyl catechol in 75 grams of dibutyl phthalate at 80° C. and pouring it into a vigorously stirred solution of 50 grams of gelatin in 50 grams of 8% aqueous saponin solution and in 500 cc. of water at 40° C.).  
 340 grams of a dispersion like dispersion A except substituting 4-methoxy-1-naphthol for 4-phenyl catechol.

This emulsion was coated on a film support and designated Coating A.

The following additions were made to one mole of a photographic emulsion of the type described above:

50 ml. of 15% aqueous saponin solution  
 660 ml. of gentisic acid (7.5% aqueous solution)  
 50 ml. of 1-phenyl-3-pyrazolidone (5% in methyl alcohol)  
 water to make a total of 4250 grams.

The treated emulsion was then coated on a film support and designated Coating B.

When processed in an alkaline activator containing sodium carbonate at a pH above 9, Coatings A and B exhibited the following sensitometric characteristics:

|                | Relative Speed | $\gamma$ | $D_{max}$ |
|----------------|----------------|----------|-----------|
| Coating A----- | 4.9            | 1.0      | 1.2       |
| Coating B----- | 5.0            | 3.0      | 2.9       |

It will be noted that Coating B exhibited a higher gamma and  $D_{max}$  than Coating A.

It was also observed that Coating A was softer and more subject to physical damage during handling than Coating B due apparently to the pressure of the oily solvent in Coating A which was necessary to disperse the 4-phenyl catechol. The need for additional gelatin in the 4-phenyl catechol dispersion also renders it difficult to obtain thin, low gelatin-containing coatings.

Coatings containing 4-phenyl catechol tend also to be more allergenic than coatings containing gentisic acid, and due to the need for the oil solvent, are more difficult to coat without running into repellancy, etc.; in addition, the incorporated 4-phenyl catechol tanning developer agent has a tendency to autoharden during storage.

*Example IV*

Coatings A and B of Example 3 above were bathed in the alkaline activator, described above, in the dark for one minute. Then the top half of each coating was ex-

posed, while in the activator, to a photoflood lamp at about 12 inches for 4 minutes. The strips were subsequently washed in 90° F. water.

The exposed half of Coating B contained an image as evidenced by an overall silver deposit, whereas, the exposed half of Coating A did not contain an image and was as clear as the unexposed bottom half. It would appear then, that the gentisic acid diffuses from the emulsion less readily than does the 4-phenyl catechol and is, therefore, available for development after the initial bathing prior to the exposure.

*Example V*

A coating was prepared as follows:

To 0.15 mole of a fine-grained 99 percent chloride orthochromatically sensitized chloroiodide emulsion (AC-1381) was added:

|                                                                             | Cubic centimeters |
|-----------------------------------------------------------------------------|-------------------|
| 15.3 percent saponin -----                                                  | 7.5               |
| 20 Semicarbazide, HCl (5 percent in distilled water at pH 5.6±0.3) -----    | 12                |
| Gentisic acid (7.5 percent in distilled water at pH 6.0) -----              | 100               |
| 25 4-methyl-1-phenyl-pyrazolidone-3 (5 percent in CH <sub>3</sub> OH) ----- | 7.5               |
| Distilled water to 642 g.                                                   |                   |

The resulting melt contained about 4.3 percent gelatin. It was coated on a cellulose triacetate film support to give 690 mg. of gelatin per square foot and 400 mg. of silver halide per square foot. The film was exposed to an image and processed in an alkaline activator containing 3 percent sodium carbonate. The non-image areas were then removed by washing in warm water. This emulsion gave an excellent negative image.

*Example VI*

When either gentisic acid or 4-methyl-1-phenyl-3-pyrazolidone were used separately as in the emulsion of Example I, there was either no image or a very faint image resulting from such use. Alone they are not highly active developing agents at the pH of the activator. The oxidation products of each developing agent, gentisic acid or 4-methyl-1-phenyl-3-pyrazolidone, are colorless and remain so even when used in combination. When 4-phenyl catechol hydroquinone, p-phenylenediamine and pyrogallol or gallic acid are used in this system, the oxidation products are colored and produce stain.

*Example VII*

Photographic emulsion as in Example I, containing the combination of gentisic acid and 4-methyl-1-phenyl-3-pyrazolidone were compared with 4-phenyl catechol incorporated in similar emulsions in alkaline activator solutions, i.e., 4 percent aqueous sodium carbonate. The developed fogged strips were washed in water at about 90° F. and the emulsion containing the 4-phenyl catechol was completely washed away, whereas the gentisic acid-pyrazolidone containing emulsion was hardened enough to remain on the film support without any reticulation or edge sloughing.

It will be appreciated that various film supports known in the art may be used such as paper, cellulose ester, plastic supports such as polyethylene, polyethylene terephthalate, etc. These supports may be oxidized, electron bombarded, etc., to improve adhesion. The silver halide emulsion may be of the usual negative type or may be a direct positive emulsion. A pigment may be added to the emulsion in order to increase the density if so desired and the support over which the emulsion is coated may have previously been subbed, coated with various coating composition to improve the hydrophilic character of the support or the like. In addition, the relief image may be subjected to various treatments known in the art to improve its receptivity to greasy printing inks or the element itself may be subjected to treatments to improve

the relative difference in attraction to greasy printing inks to improve the printability of the element for use as a printing plate.

In the accompanying drawings, I have shown a typical support at various stages in my process. As shown in FIG. 1 a support 10 is coated with a gelatino-silver halide emulsion 11 containing a substantially water soluble tanning developing agent. This material is exposed and developed by immersion in an alkaline solution to form images of silver and hardened gelatin as shown at 12 in FIG. 2. The remaining unhardened gelatin and silver halide 13 in FIG. 2 is then washed off by treatment of the support with warm water to leave images 14 of hardened gelatin on the support 10 as shown in FIG. 3.

The hydrophilic colloid is preferably gelatin, but may be any other hydrophilic colloid known in the art which is tanned by gelatin tanning agents or may be a combination of gelatin and a similar hydrophilic colloid which would provide a suitable tanning colloid layer.

Although this tanning developer combination is particularly useful in preparing a lithographic printing plate, since a silver halide emulsion incorporating this developer combination provides a hard relief image and can be coated in a relatively thin layer, it will be appreciated that this tanning developer combination may be used in other photographic applications where a tanning developer is desired to be incorporated in the emulsion. Typical emulsions where such a developer would be used are described in Yackel, U.S. Pat. No. 2,592,368, issued April 8, 1952, and Yutzy et al., U.S. Pat. No. 2,716,059, issued August 23, 1955, and the like.

Here and in the appended claims wherein it is stated that the emulsion vehicle is substantially unhardened this is defined as a meaning not harder than would be the case with gelatin containing 0.25 ounce of formaldehyde (40 percent solution diluted 1 to 3 with water) per pound, when freshly coated, or 0.1 ounce of the solution per pound for a sample aged three to six months. Emulsion layers appreciably harder are not very satisfactory for use in my process or that of the above copending application.

In general, when utilizing the usual type of photographic gelatin, useful results are obtained without addition of hardener to the emulsion. In case the gelatin in use has poor physical properties then a small amount of hardener such as formaldehyde may be used.

The emulsion layer may be exposed in the usual manner under a line drawing and is "developed" by immersion in an aqueous solution of an alkali such as sodium or potassium carbonate, an alkali metal hydroxide such as sodium hydroxide, potassium hydroxide, or ammonium hydroxide, or an amine. The addition to the alkaline solution, of other materials, is also helpful in obtaining a satisfactory relief image. For example, the addition of sodium hydroxide to a sodium carbonate solution improves the sensitometric characteristics of the material as well as the relief properties. The addition of reducing agents such as ascorbic acid, hydrazine hydrochloride, sodium sulfite, in small quantities, sodium bicarbonate and urea, are also advantageous.

After development of the exposed material in the alkaline solution, the element is washed with warm water to remove the unexposed and undeveloped colloid and silver halide and then dried. By "warm" water I means water at a temperature above 90° F. to 100° F. or higher.

It will be appreciated that the light-sensitive emulsions are prepared under normal darkroom or safelight conditions as required.

The emulsions of this invention are useful in the colloid transfer process as described in U.S. Patents 2,596,756 and 2,725,298. Development of the exposed emulsion results in hardening the exposed area of the image which then adheres to the support. The unexposed and, therefore, unhardened area is transferred to a suitable absorbent surface such as a paper receiving sheet when the emulsion is contacted against the paper receiving sheet.

The invention has been described in detail with particular reference to preferred embodiments thereof, but it will be understood that variations and modifications can be effected within the spirit and scope of the invention as described hereinabove and as defined in the appended claims.

I claim:

25 1. A process for providing a relief image comprising developing an exposed silver halide emulsion comprising a substantially unhardened gelatin vehicle and dispersed in said vehicle silver halide and a tanning developing agent comprising gentisic acid and a 3-pyrazolidone silver halide developing agent by imbibing into the gelatin vehicle an aqueous alkaline solution and removing the undeveloped silver halide containing vehicle.

2. A process of claim 1 in which the pyrazolidone is 1-phenyl-3-pyrazolidone.

35 3. A process of claim 1 in which the pyrazolidone is 4-methyl-1-phenyl-3-pyrazolidone.

4. A process of claim 1 in which the pyrazolidone is 2-acetyl-4-methyl-1-phenyl-3-pyrazolidone.

30 5. A process of claim 1 in which the undeveloped silver halide is removed by washing with warm water.

40 6. A process of claim 1 in which the undeveloped silver halide containing vehicle is transferred to an absorbent surface.

#### 45 References Cited by the Examiner

##### UNITED STATES PATENTS

2,716,059 8/1955 Yutzy et al. ----- 96—95  
50 2,751,297 6/1956 Hood et al. ----- 96—109  
3,192,046 6/1965 Kennard et al. ----- 96—95

##### OTHER REFERENCES

55 Henn et al.: Phot. Sci. and Tech. (II) 1954, pp. 126-130.

Mees: Theory of the Photographic Process 1954, MacMillan Company, New York, pp. 560 and 580-582.

NORMAN G. TORCHIN, Primary Examiner.

60 A. D. RICCI, Assistant Examiner.